

## UNITED STATES PATENT OFFICE

2,222,050

## VISCOSE LOW IN HEMICELLULOSE

Johann Joseph Stoeckly, Teltow-Seehof, and Wolfgang Linnhoff, Berlin-Lankwitz, Germany, assignors to North American Rayon Corporation, New York, N. Y., a corporation of Delaware

No Drawing. Application October 21, 1938, Serial No. 236,216. In Germany October 23, 1937

11 Claims. (Cl. 260—217)

This invention relates to a process of producing viscose which is poor in hemicellulose and solid artificial structures made thereof.

In the manufacture of artificial structures, as, for instance, artificial filaments, artificial silk and the like of viscose it has been attempted already heretofore to use for the production of the alkali cellulose a mercerizing lye which is relatively poor in hemicellulose. It is also already known that products of a higher strength in a dry and wet state are obtained, under conditions which are otherwise similar, if a cellulose pulp is used as an initial material which is of a high quality and rich in alpha cellulose. However, even when using a cellulose pulp which is rich in alpha cellulose, and pure mercerizing liquor, substantial quantities of hemicellulose are produced again in the subsequent ripening process of the alkali cellulose; therefore it has been proposed to start directly from a pulp which is so rich in alpha cellulose and of so low a viscosity that the same can be directly converted into a viscose which is poor in hemicellulose, without additional formation of hemicellulose, by mercerizing and sulphiding, avoiding the ripening of the alkali cellulose.

It is an object of the present invention to further improve and simplify this process, using ordinary commercial artificial silk pulp containing hemicellulose.

With this and further objects in view which will be apparent from the following disclosures, we use sheets of ordinary commercial artificial silk cellulose pulp containing, for example, 86 to 89% alpha cellulose which is dipped in mercerizing lye containing, for example, 18% NaOH. A conventional steeping press may be used for this purpose. The mass is then squeezed out to assume about three times its original weight or less, and then disintegrated. Ordinary mercerizing lye of technical purity or impure lye containing, for example,  $\frac{1}{2}$  to  $1\frac{1}{2}$  or more percent hemicellulose may be used. The disintegrated alkali cellulose is then ripened to a degree sufficient to attain the desired final viscosity of the viscose to be produced. Our novel process is now applied to these cellulose crumbs which have been produced after the ordinary or a special process and are more or less ripened or not ripened at all. Now, in order to clean the crumbs of alkali cellulose the same are wetted or made to a paste or dough, for example, by spraying and stirring the mass, with a limited quantity of dilute caustic soda solution of about 8-12% strength which is relatively poor in hemicellulose. After leaving

this mixture untouched advantageously for a period of one or more hours, it is squeezed out, for example, in presses of the kind used in the fat and oil industry or in the production of fruit juice. The press-cake is broken up again and the disintegrated material is made to a dough or paste with a limited quantity of mercerizing lye of, for example, 18 to 22% alkali content and of one to three times the weight of the press-cake and stirred, allowed to act for one to several hours and again squeezed out in a closed press to assume, for instance, 2.6 to 3 times the weight of the original cellulose. Now the alkali cellulose is again disintegrated and then subjected to the sulphiding process so as to be converted into viscose, in the manner known per se.

It has been found that by repeatedly steeping the cellulose into mercerizing lye of substantially more than 12% NaOH content, more particularly into the ordinary mercerizing lye of about 18% NaOH content, the so-called beta celluloses which are difficult to dissolve are dissolved from the cellulose substance only partly or not at all. However, in our process a steeping lye of 12% NaOH and less proved very well. Again, it has been found, that it is dangerous to use a lye of less than 8% NaOH content because it is difficult to reproduce in an alkali cellulose swollen with very diluted lye by a subsequent treatment with a more concentrated mercerizing lye the original state of mercerization evenly throughout the whole mass. For this reason and for safety a certain time for action is inserted between the dough-making and the squeezing operation, in order to allow for diffusion. If a washing lye or liquor of substantially less than 8% alkali content is used, it is no more possible to reproduce the degree of mercerization before, and for the purpose of, the sulphiding operation with practical mercerizing lyes and action times, and an insufficient sulphiding action and bad viscose is obtained which on account of the undissolved fibres can hardly be filtered.

The alkali cellulose of a low alkali content which has been purified with diluted lye and squeezed out, cannot be directly sulphided but, as has been found, has to be readjusted to a degree of mercerization corresponding to the higher content of alkali before the sulphiding operation.

It is an important feature of our invention that the alkali cellulose is wetted or made into a dough with a limited quantity of soda lye only, amounting to about one to three times the weight of the alkali cellulose crumbs. In this case the wetted alkali cellulose is in the form of a more or less

strongly swollen dough or paste of small volume which is still comparatively stiff and in certain cases looks almost dry. The dough does not show the known slipperiness of cellulose that has been 5 steeped into a surplus of soda lye, and is easy to squeeze out.

The wetting or dough-making by means of diluted soda lye and the squeezing out can be repeated and in the second operation a lye may 10 be used which is particularly pure, or particularly poor in hemicellulose. After the alkali cellulose has been subjected to the wetting or dough-making operation with washing lye, the pressing may be advantageously carried out under 15 a very high pressure whereby, as has been found, the subsequent readjustment or rectification by means of mercerizing lye is facilitated. Also it has been found that the press lye which has been squeezed out under the last and highest 20 pressure in one and the same pressing operation, removes the highest quantity of hemicellulose from the compressed mass. In this manner a very effective purification of the alkali cellulose can be attained.

25 The quantities of very pure lye required for the last operation are comparatively small as there are only limited quantities to be wetted or to be made to a dough and this lye is used entirely or partly for wetting or making a paste 30 in the last step but one of the process, after the squeezing operation, and then used in earlier steps of the process and finally, in an impure state, for steeping the cellulose.

35 *Example*

300 kgs. of ordinary alkali cellulose crumbs ripened for 20 hours at a temperature of 20° C. and containing about 11% hemicellulose per total amount of cellulose are made to a dough 40 with 600 kgs. of soda lye of 9% strength containing about 0.2% hemicellulose and after two hours squeezed out in a closed press to assume a weight of 280 kgs.

The alkali cellulose crumbs which have been 45 purified preliminarily are loosened in a suitable disintegrating apparatus and made to a dough with 550 kgs. of mercerizing lye of 21% NaOH and 0.1% hemicellulose, left to diffusion for two hours, and then squeezed out to assume a weight 50 of 270 kgs. The alkali cellulose is then loosened up again and sulphidized; the xanthate is dissolved to a viscose of 6.5% cellulose- and 8% alkali content.

The spinning solution of relatively high viscosity is filtered, de-aerated, left untouched for a certain period of time, if necessary, and then spun in the manner known per se with a considerable draft, which is admissible with viscose of this kind. In this manner a silk of high 60 strength in dry and wet state and of good elongation characteristics is obtained.

We are aware that many further changes may be made and numerous details of construction may be varied through a wide range without 65 departing from the principles of this invention, and we, therefore, do not purpose limiting the patent granted hereon otherwise than is necessitated by the prior art. Modifications of our invention will readily be recognized by those 70 skilled in the art, and we desire to include all such modifications coming within the scope of the appended claims. In these claims the term "moistening" is intended to cover simple moistening by spraying, etc., or kneading of the alkali 75 cellulose.

We claim:

1. The process of producing a viscose solution which comprises moistening one part by weight of an alkali cellulose selected from the group consisting of unripened alkali celluloses and ripened alkali celluloses with about one to three parts by weight of a sodium hydroxide solution containing about 8 to 12% by weight of NaOH, partly removing said 8-12% sodium hydroxide solution from said alkali cellulose by pressing, remoistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution. 10

2. The process of producing a viscose solution 20 which comprises moistening one part by weight of an unripened alkali cellulose with about one to three parts by weight of a sodium hydroxide solution containing about 8 to 12% by weight of NaOH, partly removing said 8-12% sodium hydroxide solution from said alkali cellulose by pressing, remoistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution. 25

3. The process of producing a viscose solution which comprises moistening one part of a ripened alkali cellulose with about one to three parts by weight of sodium hydroxide solution containing about 8 to 12% by weight of NaOH, partly removing said 8 to 12% sodium hydroxide solution from said alkali cellulose by pressing, re-moistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution. 40

4. The process of producing a viscose solution which comprises moistening one part by weight of an alkali cellulose selected from the group consisting of unripened alkali celluloses and ripened alkali celluloses with about one to three parts by weight of a sodium hydroxide solution containing about 8 to 12% by weight of NaOH, partly removing said 8 to 12% sodium hydroxide solution from said alkali cellulose by pressing, re-moistening the pressed alkali cellulose with said sodium hydroxide solution, partly removing said 45

8 to 12% sodium hydroxide solution by pressing, re-moistening the pressed alkali cellulose with a sodium hydroxide solution containing at least 18% by weight of NaOH, partly removing this sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution. 50

5. The process of producing a viscose solution which comprises moistening one part by weight of an unripened alkali cellulose with about one to three parts by weight of a sodium hydroxide solution containing about 8 to 12% by weight of 55

70

75

75

NaOH, partly removing said 8 to 12% sodium hydroxide solution from said alkali cellulose by pressing, re-moistening the pressed alkali cellulose with said sodium hydroxide solution, partly removing said 8 to 12% sodium hydroxide solution by pressing, re-moistening the pressed alkali cellulose with a sodium hydroxide solution containing at least 18% by weight of NaOH, partly removing this sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution.

6. The process of producing a viscose solution which comprises moistening one part by weight of a ripened alkali cellulose with about one to three parts by weight of a sodium hydroxide solution containing about 8 to 12% by weight of NaOH, partly removing said 8 to 12% sodium hydroxide solution from said alkali cellulose by pressing, re-moistening the pressed alkali cellulose with said sodium hydroxide solution, partly removing said 8 to 12% sodium hydroxide solution by pressing, re-moistening the pressed alkali cellulose with a sodium hydroxide solution containing at least 18% by weight of NaOH, partly removing this sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution.

7. The process of producing a viscose solution which comprises moistening one part by weight of an alkali cellulose selected from the group consisting of unripened alkali celluloses and ripened alkali celluloses with about one to three parts by weight of a sodium hydroxide solution containing about 8 to 12% by weight of NaOH for at least one hour, partly removing said 8 to 12% sodium hydroxide solution from said alkali cellulose by pressing, re-moistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution.

8. The process of producing a viscose solution which comprises moistening one part by weight of an unripened alkali cellulose with about one to three parts by weight of a sodium hydroxide solution containing about 8 to 12% by weight of NaOH for at least one hour, partly removing said 8 to 12% sodium hydroxide solution from said alkali cellulose by pressing, re-moistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose to form a cellulose xanthate and finally dissolving said xanthate in an alkali to form a viscose solution.

lulose with carbon bisulfide to form a cellulose xanthate and finally dissolving said xanthate in an alkali to form a viscose solution.

9. The process of producing a viscose solution which comprises moistening one part by weight of a ripened alkali cellulose with about one to three parts by weight of a sodium hydroxide solution containing about 8 to 12% by weight of NaOH for at least one hour, partly removing said 8 to 12% sodium hydroxide solution from said alkali cellulose by pressing, re-moistening the pressed alkali cellulose with a second sodium hydroxide solution containing at least 18% by weight of NaOH, partly removing said second sodium hydroxide solution by pressing to form a fluffy alkali cellulose, sulfidizing said fluffy alkali cellulose with carbon bisulfide to form a cellulose xanthate and finally dissolving said xanthate in an alkali to form a viscose solution.

10. The process of producing a viscose solution of which comprises moistening one part by weight of a ripened alkali cellulose with about one to three parts by weight of a sodium hydroxide solution containing about 8 to 12% by weight of NaOH, partly removing said 8 to 12% sodium hydroxide solution from said alkali cellulose by pressing, re-moistening the pressed alkali cellulose with a second sodium hydroxide solution containing at least 18% by weight of NaOH, partly removing said second sodium hydroxide solution from said alkali cellulose by pressing to form a fluffy alkali cellulose, sulfidizing said fluffy alkali cellulose with carbon bisulfide to form a cellulose xanthate and finally dissolving said xanthate in an alkali to form a viscose solution.

40

11. The process of producing a viscose solution low in hemicellulose content which comprises moistening for about two hours about 300 kilograms of alkali cellulose flakes containing about 11% by weight of hemicellulose with about 600 kilograms of a sodium hydroxide solution containing about 9% by weight of NaOH and 0.2% by weight of hemicellulose, pressing the moistened alkali cellulose in a closed press to a weight of 280 kilograms, loosening said pressed alkali cellulose, re-moistening said alkali cellulose with about 550 kilograms of a sodium hydroxide solution containing about 21% by weight of NaOH and 0.1% by weight of hemicellulose for about two hours, pressing said re-moistened alkali cellulose to a weight of about 270 kilograms, loosening said re-moistened, pressed alkali cellulose to form a fluffy alkali cellulose, sulfidizing said fluffy alkali cellulose to form a cellulose xanthate and finally dissolving said xanthate in an alkali to form a viscose solution.

45

55

60

JOHANN JOSEPH STOECKLY.  
WOLFGANG LINNHOFF.